

## UNITED STATES PATENT OFFICE

2,503,681

## TRANSFER RIBBON MANUFACTURE

Douglas A. Newman, Port Washington, N. Y., assignor to Columbia Ribbon and Carbon Manufacturing Company, Inc., Glen Cove, N. Y., a corporation of New York

No Drawing. Application March 26, 1946,  
Serial No. 657,332

12 Claims. (Cl. 197—172)

1

This invention relates to an improvement in the manufacturing of transfer ribbons, particularly those having a foundation of paper or paper-like material, rather than a textile fabric, with a coating of transfer composition on one surface thereof, especially a composition for making master copies for hectograph duplication.

In the manufacture of transfer ribbons of the aforesaid type, the usual procedure involves application of a transfer composition as a coating to a foundation of pliable non-textile membranous fabric of porous structure, particularly paper or paper-like materials, or a laminated structure of paper with a backing of film, e. g. of cellulose acetate or regenerated cellulose, or paper coated on its rear surface with a varnish or lacquer. The transfer composition usually contains a pigment or dye, a wax or wax-like material, softening oils or plasticizers, and in some cases, a volatile solvent. In the case of hectograph ribbons, the transfer coating composition contains a water or spirit-soluble dye, usually in crystalline form suspended in the wax-like vehicle, while in the case of ordinary transfer ribbons, pigments such as carbon black are suspended in the vehicle.

The transfer composition is applied to the paper foundation in molten or liquid state and allowed to set by cooling, or by evaporation of volatile solvent. In some of the procedures heretofore employed, the coated foundation is heated as by passing it over a heated roller, as it leaves the coating apparatus, to accelerate evaporation of solvent, or to insure uniform fusion of the coating. The foundation is usually in the form of a web of substantial width, and ribbons of suitable width for use in typewriters, hectowriters or similar devices are then cut lengthwise from the web. By reason of the inclusion of insoluble pigment or dye the transfer compositions employed as set out above are not homogeneous, and when they are applied in the ordinary manner to a foundation of the aforesaid type, they tend to form a skin or surface film of relatively sticky plasticized wax which has a tendency to stick to the guides and rollers of a typing machine. Moreover, when transfer ribbons are cut from a web of coated fabric, the cutting operation dislodges or loosens particles of the transfer composition at the edge of the ribbon and usually produces whiskers, nicks and slittings at the edge of the ribbon.

Thus, the usual method for cutting transfer ribbons of a desired width involves, first, reel-

2

ing a full-width web coated with a transfer composition on a spool, such as a tube of cardboard, placing the resulting roll on a power-driven spindle on which it is rotated, and cutting the roll at right angles to its axis by means of a power-driven rotary circular blade, into a series of spools of ribbon of desired width. A large number of spools of ribbon of desired width can be rapidly and simply produced in this manner. A fairly clean cut can be made in a roll with a well sharpened blade of perfectly circular shape, properly centered and mounted to run true in a plane perpendicular to the axis of the roll, but in practice, the cutting blade is subject to rapid deterioration, soon wearing out of round. The cutting force, being uneven, tends to cause flexure of the blade. Moreover, the blade has a flat surface facing the uncut roll, and a bevelled edge facing the ribbon being cut. Resistance to lateral displacement of the latter tends to flex the blade, accentuating unevenness in the cutting effect. As a result, particles of transfer composition are loosened or dislodged, and nicks, whiskers and slittings are formed at the edge of the ribbon, especially at the side facing the bevelled edge of the blade. Moreover, as the blade approaches the center of the roll, its peripheral speed relative to the roll increases, generating increasing amounts of heat sometimes sufficient to scorch the ribbon and further facilitating dislodgment of transfer composition. Variation in the cutting force as the blade approaches the center of the roll sets up uneven tension in the ribbon, tending to cause the transfer composition to adhere to the contiguous rear surface of the ribbon, especially when the spool is stored for a time before use.

Most of the dislodged particles of transfer composition adhere to the rear surface of the ribbon, larger amounts being present at one edge than at the other. When such transfer ribbons, especially those coated with a hectograph composition, are used in a typing device such as a typewriter or hectowriter, the dislodged or loosened particles of transfer composition are deposited on the ribbon guides and gradually build up to form pressure points which resist the intermittent feeding movement of the ribbon. Since one edge of the ribbon is usually in worse condition than the other, the pressure points develop more quickly at one side of the ribbon than at the other. During operation of the ribbon feeding mechanism, the ribbon catches at the pressure points, often tearing under the feeding tension applied thereto, particu-

larly when a nick in the edge of the ribbon is adjacent to the pressure point. Moreover, the loose particles of transfer material adhering to the ribbon become dislodged and fall on operating parts of the machine and on the copy being made, producing unsightly specks, and the hands of the operator become soiled in handling the machine, making the production of clean copies extremely difficult.

It is accordingly an object of this invention to provide a method for producing transfer coated ribbons of the aforesaid type, particularly hectograph ribbons, which do not have loosened or dislodged particles of transfer composition adhering at the edges or to the back of the ribbon, which do not have a sticky skin of wax on their surface, which do not stick to the guides or rollers of a typing machine, which do not deposit transfer composition on said guides or rollers or on other parts of the machine, and which produce clearer and sharper copies than those ordinarily obtained.

I have discovered that the foregoing disadvantages in transfer ribbons cut from a relatively wide web comprising a flexible membranous non-textile foundation of paper or paper-like material, and coated with a transfer composition containing a pigment or dye suspended in a wax or wax-like material in admixture with softening oils or plasticizers, applied with or without a volatile solvent, can be obviated either by pre-treatment of the coated web prior to cutting of the ribbon therefrom or by subsequent treatment of the ribbon.

Thus, I have found that the aforesaid disadvantages can be obviated by allowing the coated web to age for about 12 hours or longer, then subjecting it to heat treatment, e. g. by passing the web over a heated roller, at a sufficiently elevated temperature and at a suitable rate to effect fusion of the wax in the transfer coating, and then allowing the coating to solidify on cooling.

When the web is treated in this manner, and then cut into ribbons, I have found that much cleaner cuts are produced, and that displacement of particles of transfer composition at the edges of the ribbon is substantially eliminated. Moreover, the surface-film or skin of sticky wax is eliminated, so that the ribbon no longer tends to stick to the rollers or guides of a typing machine. Loose particles of the transfer composition are not deposited on the rear surface of the ribbon, and do not build up as a deposit on the ribbon guides. Hence, breakage of the ribbon during operation of the feed mechanisms of the typing device by reason of the ribbon sticking at such pressure points is avoided. In addition, I have found that impressions produced from the web, or a ribbon cut therefrom, which has been subjected to the foregoing treatment, are much clearer and sharper than those produced from the untreated web or ribbon.

While the reasons for the advantageous effect of the aging and heat treatment of this invention are not fully understood, and it is not intended to limit the invention to any theory of operation, a partial explanation may be that the aging of the web for about 12 hours or more permits the softening oils in the transfer coating to be absorbed by the paper foundation, leaving the wax and pigment in somewhat loosely cohesive condition on the surface of the foundation, the wax forming a skin on the surface of the coating. When the web is subjected, after aging, to heat treatment in accordance with my

invention so as to melt the wax, the wax in the skin is apparently absorbed into the body of the ink and forms a relatively homogeneous mass therewith having greatly improved cohesion, and 5 more uniform adhesion to the foundation. When ribbons are cut from such a web, the transfer composition does not break up at the edges, does not deposit on or stick to the rear surface of the ribbon or to the guides or rollers of the machine over which it passes, and produces clearer and sharper copies.

My invention will be more readily understood from the following example which illustrates a preferred procedure in accordance with my invention.

#### Example 1

A broad web of foundation material consisting of a layer of thin paper adhesively secured to a film of cellulose acetate or regenerated cellulose, is coated on its paper side with a hectograph transfer composition comprising essentially a wax or wax-like material such as carnauba wax, a softener such as a mineral or fatty oil or a 20 fatty substance such as lanoline, a water- or spirit-soluble dyestuff such as crystal violet in finely divided state, and if desired, a volatile solvent such as petroleum naptha. The coating is preferably applied while heating so that the 25 wax-like and oily portions thereof are liquified, and after cooling, the coated web is wound on a core, to form a roll.

The coated web is then allowed to age for about 12 hours or longer. After aging, the web 30 is unrolled, and passed progressively over a heated roller with the rear surface of the web in contact with the roller. The roller is heated at sufficiently elevated temperature over the melting point of the ink, e. g. 140° F. to 350° F., and 35 the rate of passage of the web is adjusted so as to fuse the wax contained in the coating. After leaving the heated roller, the web is allowed to cool, and is then rewound on a suitable core, e. g. a cardboard tube, to form a firm roll of substantial length and diameter. The roll is then 40 placed on a spindle on which it is rotated, and is cut at right angles to its axis into a series of 45 spools of ribbon of desired width. A circular blade, flat on one side, with its edge bevelled on the other side is employed for cutting the spools of ribbon from the roll, the blade being rotated about an axis parallel to that of the roll, and having its flat side facing the uncut portion of the roll.

The ribbons thus formed from the aged and heat-treated web are exceptionally clean, having substantially no dislodged particles of transfer composition at their edges, or on the rear surface of the ribbon. The sticky skin or surface film of wax is eliminated. In use, the ribbon passes 55 readily over the guides of a hectowriter, without deposition of transfer composition thereon to form pressure points, and without deposition on other parts of the machine. Tearing of the ribbon during use is thus practically eliminated. The ribbon can be handled for installation in the machine without substantial soiling of the hands, and the machine remains clean so that clean copies can be readily made. Moreover, the 60 transfer properties of the main body of the coating are improved by fusion of the wax occurring therein during the treatment, and sharper clearer inscriptions are produced evidently as a result of the homogenizing effect of the treatment on 65 the transfer composition.

The treatment described in the foregoing example can be applied with similar effect in the production of ribbons having a foundation of paper alone, or paper coated on its rear surface with a lacquer or varnish, or paper secured to a backing film other than cellulose acetate, e. g. to "cellophane". The advantages of the treatment are most pronounced in the case of ribbons having a hectograph transfer coating thereon, because of the rapid operation of feed mechanisms in hectowriters which increases the tendency to tear the ribbon, and because of the relatively large amount of coloring material in the transfer composition rendering deposition thereof on the machine especially obnoxious. However, the treatment of the invention can also be applied with advantage to transfer coated webs having a non-textile paper-like foundation and a pigmented coating of the kind used on ordinary carbon paper.

While the foregoing example represents a preferred procedure in accordance with my invention, variations can be made therein without departing from the scope of the invention. Thus, instead of passing the web of coated foundation over a heated roller, it can be passed through a heating zone, in which it is subjected to infra-red radiation sufficient to fuse the wax in the coating.

Moreover, I have found that ribbons having advantages similar to those obtained in the foregoing example can be secured by subjecting the ribbons to similar heat treatment after they have been cut from a roll of transfer coated web, and at least 12 hours after the transfer coating is applied to the web, to allow for aging. For example, the ribbon can be unwound from a spool cut from a roll of the coated foundation, and passed progressively over a heated roller in the same manner as in the foregoing example, or through an infra-red heating zone, so as to fuse the wax in the transfer coating. After cooling, the ribbon is rewound into a spool, substantially uniform tension being preferably maintained during rewinding.

The preferred method for heat treating the ribbon after it is cut from a roll of transfer coated foundation, comprises passing the ribbon progressively through a flame at a sufficient rate of speed to avoid scorching the ribbon, but to cause fusion of the coating composition particularly at the edge of the ribbon, to fuse particles adhering to the back of the ribbon, and to singe off whiskers, nicks and slittings along the edges thereof. In this method of treatment the ribbon is passed horizontally through a flame with its rear surface facing the source of the flame, so that the fusing effect is strongest at the edges of the ribbon. The spool of ribbon is unwound, progressively passed through the flame, and then rewound under constant tension on a suitable spool. I have found that heating ribbons and rewinding in this manner practically eliminates the development of imperfections during storage, as a result of uniformity of tension existing in the re-wound spool. Fusion of particles of transfer composition adhering to the edge and back of the ribbon substantially eliminates deposition of the particles on the ribbon guides of a machine, thus avoiding the formation of pressure points. Whiskers and slittings are largely eliminated by singeing, and the nicks are smoothed over. As a result, the danger of tearing the ribbon during passage over the guides of a typing machine upon operation of the ribbon feed is eliminated. The

spool of ribbon is clean to handle, and the machine remains clean during operation, so that the operator is not troubled by soiling the hands with transfer composition, and production of clean copies is greatly facilitated.

The following example illustrates the latter method of treating a transfer ribbon in accordance with the invention, after it has been cut from a relatively wide web of transfer-coated foundation.

#### Example 2

A web of foundation material as described in Example 1, is coated on its paper side with a hectograph transfer composition as set out in the first example; the coated web is wound on a cardboard tube as a core to form a firm roll of substantial length and diameter, and the roll is then cut into spools of ribbon in the same manner as in Example 1.

An average ribbon produced in the aforesaid manner is found on examination to have the transfer composition fractured along the edge, and loose particles thereof adhere to the back of the ribbon, or remain loose on its coated surface. Moreover, fibres of the paper or "whiskers" project from the edge, and at frequent intervals, slittings (i. e. narrow strips of the ribbon slit from the edge by slight deviation of the blade from its plane of rotation) remain. At some points, nicks are formed, constituting potential severance points. The condition of one edge of the ribbon is for the most part considerably worse in the foregoing respects than the other, because of difference in the surfaces of the cutting blade employed.

In accordance with my invention, at least 12 hours after application of the coating to the foundation, the spool of ribbon is placed on a spindle, and the end thereof attached to a second spool on which it is to be rewound, the ribbon between the spools preferably having its transfer coated surface facing upward. Rewinding is then begun, maintaining uniform tension in the ribbon between the spools. At the same time, a flame, for example, a moderately adjusted Bunsen burner flame, is applied to the ribbon as it passes from one spool to the other, the speed of the ribbon and the intensity of the flame being adjusted to avoid scorching the body of the ribbon, but at the same time, to singe off whiskers and slittings at the edge of the ribbon, and to fuse the transfer composition at least at the edges. A suitable rate of passage of the ribbon through the flame is about 10 to 50 feet per minute.

The ribbon thus treated is found on examination to be substantially free of whiskers and slittings, and nicks are smoothed out. Loose particles of transfer composition are no longer present at the edges or on the back of the ribbon, but are coalesced by fusion, and adhere firmly to the ribbon. The rewound spool is characterized by uniform tension, thus eliminating any tendency to deteriorate on standing, often inherent in the original spool because of non-uniform tension caused by the cutting operation. In use and properties, the ribbon thus treated is characterized by the same advantages as a ribbon produced according to Example 1.

When the flame treatment is applied to a ribbon after it is cut from a roll, as in Example 2, I have found further that it is possible to dispense with the aging of the coated foundation, prior to the heat treatment, without sacrificing any substantial part of the advantages characterizing the

ribbon produced in accordance with the latter example.

Variations and modifications may be made within the scope of this invention and portions of the improvements may be used without others.

I claim:

1. In the production of a transfer ribbon by coating one surface of a relatively wide strip of pliable porous non-textile membranous fabric as a foundation with a normally solid wax-containing transfer composition, and cutting said ribbon from the coated strip, the improvement which comprises aging said coating for at least 12 hours after application to said foundation, then heating said strip so as to melt the wax in the transfer composition, allowing the coating to solidify on cooling, and then cutting the strip into ribbons of relatively narrow width.

2. The method of making a spool of transfer ribbon which comprises applying a coating of a normally solid wax-containing transfer composition to one surface of a relatively wide strip of paper foundation, aging said coating for at least 12 hours after application to said foundation, passing said strip progressively through a heating zone while controlling the temperature of said zone and the rate of passage of said strip therethrough so as to melt the wax in said transfer composition, allowing the coating to solidify as said strip passes beyond said zone, winding said strip into a roll and cutting said roll at right angles to its axis to form a spool of transfer ribbon.

3. The method defined in claim 2 wherein said coating is a normally solid wax-containing hectograph transfer composition.

4. In the production of a transfer strip slit from a wider web and having a pliable, porous, non-textile membranous fabric and a coating of normally solid oleous wax-containing transfer composition on one surface of said fabric, the improvement which comprises allowing the coating to age until the oils in the coating are partially absorbed by the fabric, then heating the coating so as to melt the wax and effect the re-blending of the unabsorbed portions of the transfer composition, and cooling the coating to solidify the same.

5. The method as defined in claim 4 in which the coating of transfer material is aged and heated before the web is slit into strips.

6. The method as defined in claim 4 which includes the steps of winding the web to form a roll, slitting the roll to form spools, after which the transfer coating is aged and heated.

7. The method as defined in claim 4 in which the coating of transfer material is heated after the web is slit into strips.

8. The method as defined in claim 4 which includes the steps of winding the web to form a roll, slitting the roll to form spools of strip, aging the coating, and thereafter heating the strips by traveling the same through a flame at

a sufficient rate to singe off any whiskers or slittings on the edges of the strip and further to cause any flakes of the transfer coating clinging to the strip to be fused and, upon coalescence, to adhere to the strip.

9. In the treatment of a transfer ribbon slit from a wider strip and having a pliable, non-textile, membranous fabric, and a coating of a normally solid transfer composition on one surface of the fabric, said ribbon as a result of being slit being liable to have whiskers, slittings and nicks along an edge thereof and dislodged flakes of coating composition clinging to the back and adjacent the edges thereof, the method which comprises traveling the ribbon through a flame at a sufficient rate of speed to singe off the whiskers and slittings and fuse the coating at the edges of the ribbon to close said nicks and to adhere to the ribbon flakes clinging thereto.

10. A typewriter ribbon of the type slit from a wider web having a paper surface thereon carrying a coating of normally solid wax-containing transfer composition, the cut edges of the paper surface and coating being consolidated by said composition so that the edges are smooth and devoid of projecting paper fibers, slittings and loose flakes of transfer composition.

11. A typewriter ribbon of the type slit from a wider web having a paper surface thereon carrying a homogenized coating of normally solid wax-containing transfer composition, the cut edges of the paper surface and coating being consolidated by said composition so that the edges are smooth and devoid of projecting paper fibers, slittings and loose flakes of transfer composition.

12. A typewriter ribbon of the type slit from a wider web having a laminated foundation including a film layer and a layer of paper carrying a coating of normally solid wax-containing transfer composition, the cut edges of the film, paper and coating being consolidated by said composition so that the edges are smooth and devoid of projecting paper fibers and slittings.

45

DOUGLAS A. NEWMAN.

#### REFERENCES CITED

The following references are of record in the 50 file of this patent:

#### UNITED STATES PATENTS

| Number       | Name     | Date          |
|--------------|----------|---------------|
| 1,396,403    | Buckley  | Nov. 8, 1921  |
| 55 1,470,282 | Newman   | Oct. 9, 1923  |
| 1,533,382    | Campbell | Apr. 14, 1925 |
| 1,546,747    | Pembroke | July 21, 1925 |
| 1,700,415    | Neidich  | Jan. 29, 1929 |
| 1,772,553    | Moller   | Aug. 12, 1930 |
| 60 1,835,741 | Allen    | Dec. 8, 1931  |
| 1,913,704    | Elkan    | June 13, 1933 |
| 2,066,687    | Hudspeth | Jan. 5, 1937  |
| 2,255,104    | Dixon    | Sept. 9, 1941 |